

## UNITED STATES PATENT OFFICE

2,369,150

## LUBRICATING OIL

Bert H. Lincoln and Gordon D. Byrkit, Ponca City, Okla., assignors to Continental Oil Company, Ponca City, Okla., a corporation of Delaware

No Drawing. Application November 27, 1940,  
Serial No. 367,462

8 Claims. (Cl. 252—46)

Our invention relates to lubricating oils and more particularly to improved lubricating oils of high film strength, high resistance to oxidation, and markedly reduced formation of corrosive products during use.

This application is a continuation-in-part of our co-pending Serial No. 283,569, filed July 10, 1939.

Present-day mechanical devices require lubricating oils of high film strength, of high oiliness characteristics, and of low tendency to oxidize during use. It has been found that the present-day hydrocarbon lubricants of the very highest quality are deficient in these very important characteristics. These three properties are of vital importance under conditions of thin film lubrication where the lubricant has been squeezed from between the friction surfaces because of high pressure, slow speeds, and other causes. In modern engines, large surfaces of oil are exposed to the action of atmospheric oxygen, promoting rapid oxidation. It is readily seen that the viscosity or the body of the lubricant plays no part in thin film lubrication and that the remaining film of oil must have a very high film strength and be of high oiliness value to prevent rupture of the film of the lubricant, which would cause seizure. The oil film must tend to keep the coefficient of friction as low as possible. The oil must resist oxidation when these thin films are heated in the presence of atmospheric oxygen as they are in use.

Mechanical devices are being designed for higher pressure operation, and the film strength of the best quality straight hydrocarbon lubricant has been found to be too low for satisfactory service. It will be obvious that an invention which provides a means of improving the film strength of these lubricants is of great importance to the art of lubricant manufacture and to the designer and fabricator of mechanical devices.

Substantially all machines operate in part or at times totally under conditions of boundary or thin film lubrication, under which conditions the oiliness or unctuousness of the lubricant is the first and primary requisite of efficient operation. Those skilled in the art of lubricant manufacture or machine manufacture will readily appreciate the value of an invention that will improve the oiliness of these otherwise high-quality lubricants. Furthermore, sludge and acid are especially deleterious under conditions of thin film lubrication. The sludge is not a lubricant in any sense of the word, and the soluble acid is particularly corrosive to bearing metals such as cadmium-silver, copper-lead, and the like.

In starting idle mechanical equipment which is lubricated from a sump by pumping or cir-

culating the lubricant, there is always a short period of time in which the rubbing surfaces must operate under conditions of dry friction if ordinary hydrocarbon lubricants are used. 5 With dry friction, the wear on friction surfaces is extreme; and during cold weather when the lubricant is sluggish or during periods when the lubricating system is not functioning properly for one reason or another, rubbing surfaces may not only suffer considerable wear but may be damaged to the point where they must be replaced. The product of our invention has a very important property of reaction with the metal surfaces, penetrating or absorbing on the metal surfaces, and leaving a film of lubricant with high oiliness character, which remains on the metal surface irrespective of the length of time the machine has been idle.

This high oiliness film gives very even and 20 smooth operation, which may be easily discerned by the experienced operator or lubricating engineer.

When the hydrocarbon lubricants are diluted 25 with unburned fuel or with other light hydrocarbons, the small degree of oiliness of the original hydrocarbon lubricant is greatly decreased. We have found that the addition of the products of our invention to hydrocarbon lubricants more than compensates for the loss in oiliness and load-carrying ability from dilution.

It is well known that, in order to obtain lubricants which are preeminently satisfactory from the standpoint of oxidation in use, it is necessary to refine the oil thoroughly and then to 35 add an inhibitor of oxidation. The thorough refining may consist of many and heavy acid treatments or solvent treating so as to remove a considerable part of the oil and leave only the most stable portion. Such drastic refining is 40 necessary in order to obtain stability with respect to sludge formation, but the oil is then subject to easy oxidation to form soluble acids and other corrosive materials. This can be prevented by the addition to the refined oil of small amounts of materials which either prevent the 45 formation of these corrosive products or by some action render them inert. Furthermore, such well-refined oils are susceptible to the formation during use of lacquer-like materials which 50 tend to stick rings. This results in blow-by and hence loss of power, failure of lubrication, scratching, scoring, overheating, and eventually replacement of parts. It is practically impossible to refine a lubricant in such a manner as to avoid all three of these difficulties, namely, the formation of soluble corrosive products, sludge, and lacquer. It is considerably more advantageous to add the materials of our inven-

tion and thus avoid these difficulties by this method.

Certain compounds are adsorbed or absorbed by metals thus forming tenacious films at the surface of metals; these films are able to stand high pressures. X-ray diffraction methods have shown that compounds containing highly polar molecules, that is, molecules of unsymmetrical electrical character containing an atom or group of atoms exhibiting a secondary or residual valence, tend to produce regimentation of the molecules of hydrocarbon oil when added thereto. A metal immersed in a strongly polar compound will show a film of the compound in which there is a regimentation of molecules oriented with respect to the surface of the metal by which they are adsorbed or absorbed.

Many of our additive materials are effective when added to poorly refined or even wholly unrefined lubricants. The addends may thus be substituted in whole or in part for the usual refining processes.

In the prior art of applying these principles to the manufacture of lubricants, many diverse types of materials have been suggested to be added to obtain improvement in various characteristics. It has been found that the addition of various compounds frequently improves film strength, oxidation resistance, noncorrosiveness, and other characteristics.

One object of our invention is to provide improved inhibitors of oxidation and corrosion for addition to lubricants.

Another object of our invention is to provide film strength improving addition agents suitable for use in lubricants and especially in crankcase lubricants.

Other and further objects of our invention will appear in the course of the following description.

In general, our invention contemplates an oil of lubricating viscosity having added thereto a small amount of an organic thiocarbonate of the general formula:  $RXC(:X)XR'$  in which C represents carbon, X represents either oxygen or sulfur (at least one of the X's must be sulfur) and R and R' are organic radicals one or both of which contains carbon, hydrogen, and sulfur. The compounds here described and claimed contain extraordinarily high percentages of sulfur. Some of this sulfur is in active form and some in inactive form. The use of these compounds in lubricants provides sulfur in various forms so that under any conditions sulfur is available for its beneficial action on lubricants and as an inhibitor of oxidation. In the above formula R and R' may be aliphatic, carbocyclic, or heterocyclic in character. It is to be understood that by thiocarbonate in the appended claims we mean to include mono and trithiocarbonates as well as the dithiocarbonates.

The introduction of this additional sulfur into our thiocarbonates permits of an extraordinary flexibility in the design of the addend for a particular purpose. Thus it permits the introduction of other types of sulfur if the sulfur in the thiocarbonate is insufficient in amount or is too stable or unstable. In introducing sulfur groupings into the R's of our thiocarbonates, we do not use additional thiocarbonate groupings, since this is of no value. The additional sulfur must be in other forms in the R of our thiocarbonates.

The particular thiocarbonates of this invention have a dual action in a lubricant. One action involves increased load-carrying ability or oil-

ness, or both, while another action is directed to the stability of the lubricant. For load-carrying capacity, quantities ranging from 0.1 per cent to about 10 per cent may be added. As an anti-corrosive agent or an anti-sludging agent, or both, much smaller amounts may be required ranging from approximately 0.001 to 1.0 per cent. The action of our thiocarbonates is specific but difficult to understand. These compounds may be added to any type of hydrocarbon lubricants but show an unusual value in highly refined and solvent-treated lubricants. The blends prepared in accordance with the present invention are particularly suited for inhibiting corrosion of the new bearing metals such as cadmium-silver, copper-lead, and the like by such oils.

By oil having lubricating viscosity in the appended claims, we mean to include the so-called mineral oils and various hydrogenated, polymerized and otherwise synthetically treated oils such as volatilized oils, aluminum chloride treated oils, and the like. Furthermore, the lubricating oil may consist in whole or in part of shale oil, animal or vegetable oils such as castor oil, lard oil, corn oil, cotton seed oil, and the like.

In practice, it is better to employ compounds whose boiling point is above 225 degrees F. in order that the addition compound will not be evaporated or distilled in use. The selection of a particular compound or compounds to be used as an addition agent to the hydrocarbon or other oil is to be made considering the physical and chemical properties of the various compounds and the use to which the blend is put. Thus, if water is likely to be present during use, a substituted thiocarbonate is selected which is not affected by water. If a particular added compound proves too volatile for its application, a higher boiling material should be used and the more volatile compound used for blending in an oil intended for duty at lower temperatures. In general, for automotive crankcase lubricants, we prefer to use compounds having vapor pressures of less than atmospheric at 250 degrees F.

The following compounds are the preferred embodiment of our invention. All and each of these are examples of our invention when blended in minor proportion in an oil of lubricating viscosity. One or both of the organic radicals in our mono, di, or trithiocarbonates may be of various types as shown in the following classification. Each of the following organic or organo-metallic radical; may be combined with mono, di, and trithiocarbonate radicals as further examples of our invention, when added in minor amounts to a lubricant:

- I. Aliphatic types
  - a. Mercaptans
    1. Mercaptoamyl butoxyethoxyethylxanthate
    2. Amylxythyl mercaptomethylstearate
  - b. Sulfides and polysulfides
    3. Reaction product of sodium laurylxanthate with beta, beta prime-dichloroethyl sulfide
    4. Reaction product of sodium amyiltrithiocarbonate with dichloroamyl trisulfide
  - c. Thioacids and derivatives
    5. Reaction product of sodium amylmonothiocarbonate with methyl alpha,beta-hydroxyethylstearate
    6. Reaction product of lithium isobutylxanthate with alpha,beta-dihydroxyvaleramide
  - d. Sulfones and sulfoxides
    7. Reaction product of sodium ethoxyethylxanthate with omega-chloroamylsulfone
    8. Reaction product of sodium hexylxanthate with omega-chloroamylsulfide
  - e. Sulfurized aliphatic compounds
    9. Reaction product of potassium hexylxanthate with sulfur and chlorine-bearing methyl oleate.
    10. Reaction product of potassium ethylxanthate with sulfur chloride treated methyl linoleate
    11. Reaction product of potassium benzylxanthate with sulfur chloride treated methyl esters of soybean or corn oil acids

## II. Carbocyclic types

- a. Mercaptans and thiophenols
  - 12. Mercapto-dodecaphydro-diphenyl ethylxanthate
  - 13. Reaction product of potassium butyl-mono-thiocarbonate and o-chlorophenyl ethylmercaptan
- b. Sulfides and polysulfides
  - 14. Reaction product of chlorobenzyl disulfide and potassium hexyltrithiocarbonate
  - 15. Reaction product of sodium amyltrithiocarbonate and chlorophenylethyl disulfide
  - 16. Reaction product of sodium amyl-mono-thiocarbonate with chlorodiphenyltrisulfide
  - 17. Reaction product of potassium amylxanthate with chlorodiphenylsulfide
- c. Thioacids and derivatives
  - 18. Reaction product of sodium laurylxanthate with omega-chlorothiobutanoic acid
  - 19. Reaction product of sodium benzylxanthate with alpha-bromothiobutyramide
- d. Sulfones and sulfoxides
  - 20. Reaction product of potassium octadecylxanthate with chlorodiphenylsulfone
  - 21. Reaction product of potassium ethyltrithiocarbonate with chlorodibenzylsulfone
  - 22. Reaction product of sodium ethylmono-thiocarbonate with chlorodibenzylsulfoxide

## III. Heterocyclic types

- 23. Reaction product of chlorohydroxythiophene with sodium butoxyethylxanthate
- 24. Reaction product of potassium ethoxyethylxanthate with chlorothianthrene

The other members of the classes represented may be used within the scope of our invention.

The thiocarbonates have varying degrees of solubility in hydrocarbon and other oils. In some cases it is necessary to use a solvent for the compound or to form colloidal suspensions of the compound in oil. While some of these compounds have only limited solubility in hydrocarbon oils, it is to be remembered that because of their great efficiency extremely small amounts are often effective. Thus we have used as little as 0.001 per cent of some of these compounds, and it will be seen that a difficultly soluble material may dissolve to a sufficient extent to be satisfactory for our purpose. In general, more than 0.001 per cent of our addition agents are used; and we may add one, two, or even five per cent or more.

Furthermore, it is well known that different types of oils have different capabilities of dissolving a given material. For some purposes therefore, we prefer paraffinic, for other purposes, asphaltic, and for still other purposes, naphthenic or mixed base lubricants. Another method of obtaining a satisfactory mixture of addition agent with the hydrocarbon oil is the use of a mutual solvent to bring the addend into solution. Alternatively, peptizing agents may be added to maintain the substituted thiocarbonate in permanent suspension.

Many of the more difficultly soluble materials are rendered more soluble by the introduction of alkyl groups, particularly those containing four or more carbon atoms. The isoamyl, octyl, lauryl, and octadecyl radicals and radicals from paraffin wax greatly increase the solubility of organic compounds in oil. One or more of such groups may be introduced as required.

It is sometimes advantageous to combine more than one of these compounds in a blend to obtain particular properties. We accomplish this by mixing two or more of these compounds together and blending the mixture with the hydrocarbon oil or by blending one in the hydrocarbon oil, blending the second into this mixture, and so on until the composition is complete.

The various thiocarbonates improve both the film strength and oxidation characteristics of the hydrocarbon oil. For example, the sludging tendencies may be decreased by as little as 0.001 per cent of our thiocarbonates. The oxidation characteristics of lubricants are very important, and these are markedly improved by our com-

pounds. The ability to reduce friction is another feature contributed to lubricants by some of our compounds.

It may be desirable to include in one and the same blend, in addition to the addends here described, other addends for specific purposes. Thus, we may add a pour point depressor such as a naphthalenechlor wax condensation product, a viscosity index improver such as certain resins or polymerized hydrocarbons, and sulfur or phosphorus-containing inhibitors, in addition to our thiocarbonates. Furthermore, various metallic compounds may be added to the blend without interfering with the action of our ingredients. Indeed, in some cases it is advantageous to combine with our thiocarbonate compounds in a hydrocarbon oil blend such materials as calcium dichloro-stearate, chromium oleate, aluminum stearate, and other metallic soaps. Various halogenated oxygen-bearing ring or aliphatic compounds may be added, such as methyl dichlorostearate, chlorodiphenylene oxide and the like.

Other examples of halogen and phosphorus-containing organic compounds which we may use advantageously in conjunction with our thiocarbonates include chlorinated paraffin wax chlorinated diphenyl, chlorinated naphthalene, chlorinated diphenyl ether, dichloropropyl ether, epichlorohydrin, octadecyl trichloroacetal, chlorobutyron, o-chloroacetophenone, trichlorobenzophenone, dichlorostearic acid, calcium dichlorostearate, dichlorostearamide, o-chlorostearanilide, pentachlorophenyl benzoate, a chlorinated wax-diphenyl condensation product containing residual chlorine, trichlorophenyl, trichloroaniline, chlorophenylstearic acid, chlorobenzanilide, chlorophenyl phosphate, tricresyl phosphate, chlorophenyl phosphine, cresyl phosphite, phosphazine, phosphanilide, phosphazobenzene, phosphorus isothiocyanide, phosphoryl isothiocyanide and the like. In general, any halogen or phosphorus-bearing organic compound having a vapor pressure of less than atmospheric at 140 degrees C. has been found suitable as an auxiliary addition agent to our sulfurized compounds.

Our addends are admirably adapted for use in lubricating oils of all types including those designed for use in automotive crankcases, Diesel oils, and any other oils of lubricating viscosity. Furthermore, our addends are advantageously blended in gasoline and other petroleum fuels either directly or after being blended first in a lubricating oil and then added to the fuel. Soap-thickened mineral oils of all types ranging from those showing only a slight increase in viscosity over that of the mineral oil alone to the semi-solid and solid greases containing fifty per cent or more of soap are amenable to treatment according to our invention. In making these greases, the usual soaps such as sodium stearate, aluminum stearate, calcium soaps of beta fat, and the like may be used to form the large part of the necessary soap. Various other thickening ingredients or materials for other purposes may be added. These include yarn, hair, graphite, glycerol, water, lampblack, mica, zinc dust, litharge, and the like.

In making a lubricating gasoline, we blend 0.5 per cent of a blend of a substituted thiocarbonate in oil with gasoline. It is to be understood, however, that the hydrocarbon oil in the treated fuels may be of a viscosity of from about 35 seconds at 100° F. S. S. U. to 350 seconds or more and the

amount of oil blended with the thiocarbonate to form the fuel addend may vary between 0 and 99.5 per cent. In some cases the fuel may be prepared without adding any hydrocarbon oil. The quantity of thiocarbonate in the final blended fuel may vary from 0.001 to 1.0 per cent or slightly more.

It will be understood that certain features and sub-combinations may be employed without reference to other species or combinations. This is contemplated by and is within the scope of our claims. It is further obvious that various changes may be made in details within the scope of our claims without departing from the spirit of our invention. It is therefore to be understood that our invention is not to be limited to the details described.

Having thus described our invention, we claim:

1. A lubricant comprising a major proportion of oil of lubricating viscosity and a minor proportion of an organic thiocarbonate of the formula



in which at least one X represents sulfur and the other X's represent oxygen and in which R and R' represent organic radicals at least one of which contains carbon, hydrogen and sulfur said sulfur being present in the form of a sulfide, polysulfide, mercaptan, thio acid, sulfone, sulfoxide, or as a sulfurized organic radical prepared by treatment with elemental sulfur.

2. A lubricant comprising a major proportion of oil of lubricating viscosity and a minor proportion of an organic thiocarbonate of the formula



in which at least one X represents sulfur and the other X's represent oxygen and in which R and R' represent organic radicals containing carbon, hydrogen and sulfur said sulfur being present in the form of a sulfide, polysulfide, mercaptan, thio acid, sulfone, sulfoxide, or as a sulfurized organic radical prepared by treatment with elemental sulfur.

3. A lubricant comprising a major proportion of oil of lubricating viscosity and a minor proportion of an organic xanthate of the formula



in which R and R' represent organic radicals at least one of which contains carbon, hydrogen and sulfur said sulfur being present in the form of a sulfide, polysulfide, mercaptan, thio acid, sulfone, sulfoxide, or as a sulfurized organic radical prepared by treatment with elemental sulfur.

5 4. A lubricant comprising a major proportion of oil of lubricating viscosity and a minor proportion of an organic xanthate of the formula



in which R and R' represent organic radicals containing carbon, hydrogen and sulfur said sulfur being present in the form of a sulfide, polysulfide, mercaptan, thio acid, sulfone, sulfoxide, or as a sulfurized organic radical prepared by treatment with elemental sulfur.

15 5. A lubricant comprising a major proportion of oil of lubricating viscosity and a minor proportion of the reaction product of potassium amylyxanthate and chlorodiphenylsulfide.

20 6. A lubricant comprising a major proportion of oil of lubricating viscosity and a minor proportion of the reaction product of sodium laurylxanthate with beta, beta prime dichloroethyl sulfide.

25 7. A lubricant comprising a major proportion of oil of lubricating viscosity and a minor proportion of the reaction product of chlorobenzyl disulfide and potassium hexyltrihiocarbonate.

30 8. A lubricant comprising a major proportion of oil of lubricating viscosity and a minor proportion of an organic thiocarbonate of the formula



35 in which at least one X represents sulfur and the other X's represent oxygen and in which R and R' represent organic radicals, at least one of which contains carbon, hydrogen, and sulfur, said sulfur being present in the form of a sulfide, polysulfide, mercaptan, thio acid, sulfone, sulfoxide or as a sulfurized organic radical prepared by treatment with a sulfurizing agent selected from the group consisting of elemental sulfur and a sulfur compound.